

June 13, 1950

A. B. JENNINGS

2,511,112

PROCESS FOR OBTAINING COLOR SEPARATIONS  
FROM MULTILAYER PHOTOGRAPHIC FILM  
Filed Sept. 12, 1945

*Fig. 1.*

RED      GREEN      BLUE



*Fig. 2.*



INVENTOR.

*Andrew Bradshaw Jennings*  
BY

*Lynn Barrett Morris*  
ATTORNEY

## UNITED STATES PATENT OFFICE

2,511,112

## PROCESS FOR OBTAINING COLOR SEPARATIONS FROM MULTILAYER PHOTOGRAPHIC FILM

Andrew Bradshaw Jennings, New Brunswick, N. J., assignor to E. I. du Pont de Nemours & Company, Wilmington, Del., a corporation of Delaware

Application September 12, 1945, Serial No. 615,773

6 Claims. (Cl. 95—2)

1

This invention relates to color photography and more particularly to photographic films and processes of producing color separation records therefrom. More particularly it relates to bipack photographic films, one of the film elements of which will record two different color separation records and to processes for obtaining individual color separation records therefrom.

An object of this invention is to provide new and useful multipack photographic films. A further object is to provide bipack films for recording three-color separation records which can be utilized to readily reproduce three individual color separation records. A still further object is to provide a bipack film with one element for recording two color separation records from which one record can readily be removed in a reproduction process. Another object is to provide novel processes for obtaining color separation records from such a bipack. Still other objects will be apparent from the following description of the invention.

It has been found that novel bipack photographic films which are relatively easy to manufacture and can be readily processed to three-color separation negatives with existing equipment and facilities of commercial motion picture laboratories by the following methods.

The front film for the novel bipack is made by coating a suitable film base on one side with a water-permeable colloid-silver halide emulsion, a layer of such a colloid free from light-sensitive silver salts is then coated on the resulting layer after it has dried, then there is coated on the latter colloid layer, a layer of a water-permeable colloid-silver halide emulsion. The respective silver halide layers are so disposed and/or sensitized that each is sensitive to a different primary color region of the visible spectrum. The innermost layer is generally sensitive to blue light, whereas the outermost layer may be sensitive, in addition, to green or red light. A light screening dye or pigment is either placed in the innermost layer or in the intermediate layer free from silver halides. For example, either the blue-sensitive layer or the screening layer contain colloidal silver and it is preferably yellow in color so that it has blue light absorption characteristics and will allow green and red light to expose the remaining layers. Other types of colloidal or inert silver may be used, however, in conjunction with a yellow filter dye which may be placed in the emulsion or separator layer.

The rear film for the novel bipack merely consists of a transparent film base which carries

2

a light-sensitive silver halide water-permeable colloid emulsion layer. The emulsion layer is sensitive to red or green light.

In using the film, the two emulsion surfaces of the front film element A and the rear film element B are placed in a camera so that the front film is first exposed through the base. The two films are then developed whereby three-color separation records are formed in the respective layers. The front film color separation records are then separated by printing a master positive C of both records as shown in Fig. 1 of the attached drawing. The green record is removed from the original negative A by immersion in hot water or an aqueous solution of an alkaline thiocyanate, e. g., sodium, potassium, and ammonium thiocyanates; chlorohydrins, e. g., ethylene chlorohydrins; amides, e. g., acetamide, hydroxyacetamide, etc.

If desired, a hardening developer solution may be used in the development of the front film. If a normal developer is used, a hardening bath can be used prior or during the removal of the green record. After removal of such record, the master positive C and the positive blue record are superimposed and a "dupe" negative E is printed therefrom.

In the preferred aspect of the invention, a novel front film element is made, as shown in Fig. 2, by depositing on a transparent film base 1 a blue-sensitive gelatino-silver halide emulsion having dispersed therethrough yellow colloidal silver to form layer 2. Next there is coated a layer 3 composed of gelatin upon which is deposited an ortho-sensitized gelatino-silver halide emulsion to form layer 4. The film element just described is placed in contact with a film element having a panchromatic gelatino-silver halide emulsion layer, as described above and exposed to a color scene.

The film elements are developed in an ordinary developer, fixed, washed, and dried. A master positive C is then printed as shown in Fig. 1. The film element is then treated in an aqueous solution containing ammonium dichromate and potassium thiocyanate. They may be used in respective amounts of 50 to 200 and 20 to 100 per liter of solution. It has been found that the solution hardens the gelatin layer containing the dispersed silver but does not bleach the silver images.

In addition, the solution softens the separator layer so that the outer layer can more easily be removed. Upon rinsing the film in water, the separator layer of plain gelatin is dissolved which permits easy removal of the outer green-sensitive layer. The surface of the blue-sensitive emulsion

layer is substantially unaffected by the treatment which is somewhat surprising and unexpected because in the absence of the colloidal silver the surface has a relief image.

Colloidal yellow silver may be used in the gelatin separator layer if desired but when so used is not as satisfactory. It is more difficult to remove the separator layer and outer image bearing layer. There is formed, moreover, a relief image surface on each of the emulsion layers.

The yellow colloidal silver can be made by adding solution B to A (which follow) at a temperature of 80° F. slowly with stirring:

*Solution A*

|                              | Grams |
|------------------------------|-------|
| AgNO <sub>3</sub> (crystals) | 20    |
| Gelatin                      | 150   |
| Water                        | 2000  |

*Solution B*

|                            |         |        |
|----------------------------|---------|--------|
| Diphenyl carbazide         | grams.. | 7.28   |
| Ethanol                    | ccs..   | 728.00 |
| NH <sub>4</sub> OH (conc.) | drops.. | 12.00  |

The resulting solution was set by cooling and was pressed through a die to form noodles which were cut into short lengths and washed several times. Still other methods for making yellow colloidal silver and dispersions thereof are described in copending application Serial No. 590,390, filed April 26, 1945, now abandoned, and can be used in carrying out the present invention.

The invention will be further illustrated by the following exemplary procedures, but it is not to be limited to them.

*Example I*

A cellulose nitrate film base having a thin gelatin coating was coated with a gelatino-silver iodobromide emulsion which had admixed therewith 50% of yellow colloidal silver prepared as described above, to a weight of 52 mg. per sq. dec. After drying a gelatin solution containing 629 g. of gelatin per 15,000 g. of water was digested 15 minutes at 125° F., cooled to 100° F. and coated to form a layer .0001 inch thick. A gelatino-silver iodobromide emulsion containing 1,1'-diethyl-2,2'-cyanine iodide as an ortho-sensitizing dye was coated on the gelatin layer to a weight of 48 mg. per sq. dec. A gelatin solution containing 450 g. of gelatin per 14,400 g. of water was coated in like manner to form a thin anti-abrasion layer. This film element constitutes the front film A of a bipack.

A similar film base was coated with an aqueous gelatin solution to a weight of 50 mg. per sq. dec. and dried. A gelatino-silver iodobromide emulsion containing as a green blind sensitizing dye 1,1'-diethyl-2,4'-carbocyanine iodide was coated on the gelatin substratum. It constituted the rear film of a bipack.

The two films were placed with the gelatin layers in contact and exposed to a color scene and processed as follows:

(1) Developed for ten minutes in the following developer:

|                           |         |      |
|---------------------------|---------|------|
| Hydroquinone              | grams.. | 7.5  |
| Metol                     | do..    | 5.0  |
| Sodium sulfite (anhyd.)   | do..    | 60.0 |
| Sodium carbonate (anhyd.) | do..    | 50.0 |
| Potassium bromide         | do..    | 4.5  |
| Water                     | liter.. | 1.0  |

(2) Fixed in the following solution and washed and dried:

|                         |         |     |
|-------------------------|---------|-----|
| Water                   | ccs..   | 500 |
| Hypo                    | grams.. | 240 |
| Sodium sulfite (anhyd.) | do..    | 10  |
| Sodium bisulfite        | do..    | 25  |

5 Water to liter.. 1

(3) Film A was then bleached for 5 minutes at 65° F. in a solution made by adding to 60 cc. of water 10 cc. of Solution A and 10 cc. of Solution B which follow:

*Solution A*

|                       |         |    |
|-----------------------|---------|----|
| Sulfuric acid (conc.) | ccs..   | 4  |
| Ammonium dichromate   | grams.. | 20 |
| Water to              | liter.. | 1  |

*Solution B*

|                 |         |    |
|-----------------|---------|----|
| Sodium chloride | grams.. | 45 |
| Water to        | liter.. | 1  |

20 (4) Washed 5 minutes in hot water at 115° F. whereby the gelatin separator dissolved and the green-sensitive layer was removed.

(5) Redeveloped 5 minutes in the following developer:

*A*

|                         |         |      |
|-------------------------|---------|------|
| Sodium sulfite (anhyd.) | grams.. | 6.5  |
| Pyro                    | do..    | 28.3 |
| Potassium bromide       | do..    | 6.5  |
| Water to                | liter.. | 1.0  |

*B*

|                                |         |       |
|--------------------------------|---------|-------|
| Sodium carbonate (monohydrate) | grams.. | 113.4 |
| Water to                       | liter.. | 1.0   |

*C*

|                  |         |      |
|------------------|---------|------|
| Sodium bisulfite | grams.. | 85.0 |
| Water to         | liter.. | 1.0  |

40 For use take:

|                          |  |
|--------------------------|--|
| 75 cc. A                 |  |
| 75 cc. B                 |  |
| 100 cc. H <sub>2</sub> O |  |

45 In place of step (4) the outer layer can be removed by using any of the gelatin solubilizing agents above mentioned. For example, after developing and printing the master positive, the front film is bathed at 68° F. in a solution of ammonium thiocyanate (200 g.) in water (1 liter).

50 The outer layer and separator soften and float away. After washing the remaining blue record is dried. The elimination of the green record required only three minutes.

55

*Example II*

A bipack film element as described in Example I was exposed to a color scene and the front film was processed as follows:

60 (1) Developed 10 minutes in:

*A*

|                         |         |      |
|-------------------------|---------|------|
| Sodium sulfite (anhyd.) | grams.. | 6.5  |
| Pyro                    | do..    | 28.3 |
| Potassium bromide       | do..    | 6.5  |
| Water to                | liter.. | 1.0  |

*B*

|                                 |         |       |
|---------------------------------|---------|-------|
| Sodium carbonate (mono-hydrate) | grams.. | 113.4 |
| Water to                        | liter.. | 1.0   |

*C*

|                  |         |      |
|------------------|---------|------|
| Sodium bisulfite | grams.. | 85.0 |
| Water to         | liter.. | 1.0  |

For use take:

75 cc. A  
75 cc. B  
100 cc. H<sub>2</sub>O

- (2) Fixed as in Example I.
- (3) Washed and dried.
- (4) Washed 5 minutes in water at 110° F., rinsed and dried.

*Example III*

A photographic film as described in Example I was developed and fixed after the manner described in steps (1) and (2) thereof. The film was then treated at room temperature in an aqueous solution containing 50 to 200 parts of ammonium dichromate and 20 to 100 parts of potassium thiocyanate per liter, whereby the outer layer was removed and then rinsed in plain water and dried. This method eliminates redevelopment.

*Example IV*

A photographic film as described in Example I was developed and fixed after the manner described in steps (1) and (2) thereof. The film was then treated in an aqueous solution containing 50 to 200 parts of ammonium dichromate per liter and next treated in an aqueous solution containing 20 to 100 parts of potassium thiocyanate whereby the outer layer was softened and removed. The film was then rinsed in water at room temperature and dried.

While the novel element containing two light-sensitive layers and a stratum of colloidal silver has been described as the front element of a bipack, it is not limited to such an arrangement but can be the rear element if desired.

An advantage of the present invention is that it enables the photographic technician to produce three-color separation negatives of high quality in a shorter time and utilizing the existing equipment and facilities of the commercial laboratory.

Another advantage resides in the fact that after the green record is removed from the front negative bipack film the blue record retains its original character, especially when the colloidal silver is disposed in such layer.

A further advantage is that photographic processing time is decreased and quality is enhanced by the simple expedient of using colloidal silver in an inner silver halide emulsion layer or a contacting light-in-sensitive water-permeable colloid layer.

The type of material lends itself to use in ordinary ciné cameras with the usual bipack modifications.

The preferred aspect permits use of solutions at a normal processing temperature thereby reducing the distortion characteristic of high temperature processing.

As many widely different embodiments of this invention can be made without departing from the spirit and scope thereof, it is to be understood that the invention is not to be limited except as defined by the claims.

What is claimed is:

1. The process which comprises developing an exposed photographic element comprising a transparent film base having superimposed thereon in order a water-permeable gelatin silver halide layer which is sensitive to blue light and contains yellow colloidal silver, a water-permeable light-insensitive gelatin layer, and a water-permeable silver halide layer which

is sensitive to a different primary color of the visible spectrum, fixing said element and removing said light-insensitive layer and outer light-sensitive layer by treatment in an aqueous bath, said process being further characterized in that prior to removing said layers the element is treated in an aqueous bath containing a gelatin hardening agent which reacts with the colloidal silver in the blue-sensitive layer to uniformly harden the gelatin of said layer.

2. The process which comprises developing an exposed photographic element comprising a transparent film base having superimposed thereon in order a blue-sensitive gelatin silver halide emulsion layer containing yellow colloidal silver, a light-insensitive gelatin layer and a gelatin-silver halide emulsion layer which is sensitive to a primary color of the visible spectrum higher than blue, fixing said element and removing said light-insensitive layer and outer light-sensitive layer by treatment in a hot aqueous bath, said process being further characterized in that prior to removing said layers the element is treated in an aqueous bath containing a soluble dichromate gelatin hardening agent which reacts with the colloidal silver in the blue-sensitive layer to uniformly harden the gelatin of said layer.

3. The process which comprises developing an exposed photographic element comprising a transparent film base having superimposed thereon in order a water-permeable gelatin silver halide layer which is sensitive to blue light and contains yellow colloidal silver, a water-permeable light-insensitive gelatin layer, and a water-permeable light-insensitive colloid layer, and a water-permeable silver halide layer which is sensitive to a primary color of the visible spectrum higher than blue, fixing said element, treating the fixed element in an aqueous solution of ammonium dichromate and potassium thiocyanate which react with the colloidal silver in the blue-sensitive layer to uniformly harden the gelatin of such layer, and rinsing the treated element in water whereby the separator and outer developer layer are removed.

4. The process which comprises developing an exposed photographic element comprising a transparent film base having superimposed thereon in order a water-permeable gelatin silver halide layer which is sensitive to blue light and contains yellow colloidal silver, a water-permeable light-insensitive gelatin layer, and a water-permeable silver halide layer which is sensitive to a primary color of the visible spectrum higher than blue, fixing said element, treating the fixed element in an aqueous solution of ammonium dichromate and then in an aqueous solution containing potassium thiocyanate which react with the colloidal silver in the blue-sensitive layer to uniformly harden the gelatin of such layer, and rinsing the treated element in water whereby the separator and outer developed layer are removed.

5. The process which comprises developing an exposed photographic element comprising a transparent film base having superimposed thereon in order a blue-sensitive gelatin silver halide emulsion layer containing yellow colloidal silver, a light-insensitive gelatin layer, and a gelatin-silver halide emulsion layer which is sensitive to a primary color of the visible spectrum higher than blue, fixing said element, treating the fixed element in an aqueous solution of ammonium dichromate and potassium thiocyanate which react with the colloidal silver in the blue-sensitive layer to uniformly harden the gelatin of such layer,

and rinsing the treated element in water whereby the separator and outer developed layer are removed.

6. A process as set forth in claim 3 wherein the ammonium dichromate is present in an amount of 50 to 200 grams and the potassium thiocyanate is present in an amount of 20 to 100 grams per liter of solution.

ANDREW BRADSHAW JENNINGS.

REFERENCES CITED

The following references are of record in the file of this patent:

UNITED STATES PATENTS

| Number       | Name            | Date          |
|--------------|-----------------|---------------|
| Re. 18,680   | Troland         | Dec. 6, 1932  |
| 1,958,830    | Lierg           | May 15, 1934  |
| 5 2,153,617  | Eggert et al.   | Apr. 11, 1939 |
| 2,172,262    | Schinzel        | Sept. 5, 1939 |
| 2,191,502    | Sease et al.    | Feb. 27, 1940 |
| 2,220,187    | Wilmanns et al. | Nov. 5, 1940  |
| 2,241,519    | Pollak          | May 13, 1941  |
| 10 2,262,055 | Sease et al.    | Nov. 11, 1941 |
| 2,266,443    | Schinzel        | Dec. 16, 1941 |
| 2,295,013    | Schinzel        | Sept. 8, 1942 |
| 2,316,782    | Gaspar          | Apr. 20, 1943 |
| 2,320,418    | Eggert et al.   | June 1, 1943  |